

May 19, 1936.

J. A. DE CEW

2,041,285

PAPER SIZING

Filed Sept. 28, 1933



INVENTOR.

JUDSON A. DECEW

*Judson A. DeCew*

ATTORNEY.

## UNITED STATES PATENT OFFICE

2,041,285

## PAPER SIZING

Judson A. De Cew, Mount Vernon, N. Y.

Application September 28, 1933, Serial No. 691,420

10 Claims. (Cl. 92--21)

This invention relates to paper sizing which is a complicated operation on account of the varied conditions under which paper is made. Paper sizing consists primarily in the preparation of a 5 sizing material consisting chiefly of rosin and soda in the form of a partially saponified solution or emulsion which becomes effective as a sizing agent after it has been acidified by an acid salt such as sulphate of alumina. The essential 10 ingredients that produce the effect called sizing, are rosin and alumina, which may be combined in innumerable ways to produce different degrees of water resistance or no sizing effect whatever.

The chemical composition and the physical 15 form of the rosin emulsions and the chemical analysis of the coagulant have a bearing upon the sizing results but these are not the most important factors in the sizing process, because they can be made to react upon each other in such a 20 manner as to produce good sizing results, a partial sizing result or no sizing.

The important factors in sizing paper are that the resinous material be spread uniformly over 25 the surface of the fibers; that it be precipitated thereon with the alum solutions in a manner to give the material its maximum colloidal property; that these colloidal properties be not destroyed before the stock reaches the paper machine; that all alkalinity of the precipitate must be removed 30 and the precipitate must not be acidified to such a degree that its properties will be destroyed when the paper is being dried where the heat of the driers can decompose the excess alum solution into free acid and alumina.

35 Paper can be sized with rosin and alum in so many ways with different degrees of efficiency that there are many unexpected results that have never been properly understood or explained. For instance, while it has been known that all 40 uncoagulated sizing materials containing rosin are alkaline and in the form in which they are mixed with the paper stock they contain free alkali, and that some sizing materials have more free alkali than others, still the majority of paper 45 mills first add their size and then the alum in the beaters. Thus it has not been made known or appreciated before that when the size is added to a neutral pulp in a beater the free alkali is absorbed by the pulp and, the amount of alum required to size the paper does not depend upon 50 the reaction between the alum and the size, but is governed by the acidity required to remove the alkali from the fiber under the conditions of temperature, concentration and time for reaction 55 that exist.

This is the normal condition in sizing practice and therefore, the average mill is obliged to use from two to three times the amount of alum actually required to size the paper. But the mill operator finds that if the alum is reduced, 5 the fibers remain alkaline and the paper is unsized. If the mill happens to be following the practice that occasionally exists, of adding the alum first, and then the rosin size, it obtains the following results: if the size emulsion is added to 10 the paper stock in the beater after the alum, it is immediately coagulated locally at the point at which it is added, and the precipitated size is then distributed by mixing with the rest of the pulp. In most cases where this is done, there is 15 no sizing effect produced in the paper, but in some cases a sizing effect can be obtained if the size is mixed with the stock quickly enough, such as would be obtained by the mixing action of a Jordan, but only by the use of more rosin than 20 should be required.

The value of a sizing process does not depend upon whether or not it sizes paper but upon whether it sizes paper in a wasteful or in an 25 economic manner. So, among others, one object of this invention is to reduce the amount of alum used in sizing paper. The invention is based upon my discovery that the efficiency of the sizing can be improved by adding the sizing ingredients 30 to the paper in a way that produces certain new chemical reactions that produce the highest efficiency in the sizing of paper. The process of this invention eliminates the danger of the size being coagulated before it is mixed with the stock. It brings about the sizing reaction rapidly and 35 under controlled acidities and time factors and in a degree of concentration of paper stock that enables the reaction to be completed before the stock passes to the paper machine.

The essential part of this invention is considered 40 to be the continuous mixing of the size with the pulp before coagulation thereof under conditions which do not allow time for the free alkali in the size to be absorbed by the pulp fibers, and the rapid coagulation of the size onto the 45 fibers by adding it to an alum solution mixed with fibers where the pH of such alum solution is controlled within certain limits.

For the better understanding of how this invention 50 may be carried out the drawing accompanying this specification shows diagrammatically a flow sheet of a paper sizing plant, on which legends are used to indicate the various pieces of usual equipment commonly found in a paper mill.

That is, the drawing shows a typical paper sizing plant having a beater, a beater chest, a machine chest, a machine head box, a screen, a breast roll and paper machine, all as is usual. 5 Such a plant may or may not have a Jordan which if used would be located between the beater chest and the machine chest. For the purpose of easy identification, a Jordan is indicated in the drawing. However, the Jordan is neither a part of 10 nor necessary to this invention but is shown merely to illustrate the continuous sequence in a flow sheet of an ordinary paper mill. The invention could be illustrated just as well by showing the beater chest head box or the Jordan head box 15 as it is labeled directly connected to the machine chest and head box of the paper machine without any Jordan being present. The novel features of the invention reside in the relationship of the special chemical reactions obtained by the sequence of operations described. 20

The process may be practiced by adding a stream of sizing emulsion or solution to the stream of slightly acidified or neutral pulp in a manner whereby these materials are mixed together as 25 they pass from the beater chest to the machine chest. The alum solution is added continuously to the machine chest where it becomes diluted and mixed with the stock and the precipitated size. The sizing reaction is continuous inasmuch 30 as the mixture of size and paper stock are continually reacting in the machine chest with the mixture consisting of (1) acidified fibers, (2) acidified sizing precipitates and (3) diluted alum solution made basic by its continuous reaction 35 with the size.

This is an entirely new sizing reaction to be made use of knowingly. It involves a new combination of conditions that can be maintained consistently and that is entirely independent of 40 the existence of a Jordan in the paper mill, although the reactions should take place within certain limits. These limitations are that the size must be mixed with the pulp without coagulation. If the mixture of size with the acidified 45 or neutral pulp is alkaline, then the size should be coagulated before the fibers have time to become alkaline. The reaction with the alum takes place in the undiluted stock in the machine chest. The size is not precipitated directly by the fresh 50 alum solution, but by a partially acidified mixture of fibers and precipitated rosin size and an alum solution having a pH of over 4.

More particularly, just sufficient alum or paper-machine water is added to the paper stock in the beater to remove all alkalinity from the fibers. 55 If they are already acidified by prior treatment, this is not required. The coloring matter may be added to the stock in the beater, but not the sizing ingredients. After being beaten, the stock is discharged into a chest called the beater chest. From here, it is pumped to a head box where it flows by gravity to a Jordan if used and if not used it is discharged into a pipe carrying it to the machine chest. 60

In carrying out my process, the size is mixed with the pulp at some point in its continuous flow from the beater chest to the machine chest. The size emulsion is added in a continuous stream, after the stock leaves the beater chest. As there 65 is not sufficient acidity in the pulp to coagulate the size it is not material at which point it is added, as long as the fibers do not become alkaline from contact with the size. The time of contact can be regulated to avoid this. The mixture of pulp and uncoagulated size is then dis- 70

charged into the machine chest. The alum for coagulating the size is discharged in a continuous stream into the machine or coagulation chest, where it maintains the acidity required for the chemical reaction. Ordinary commercial alum 5 has an acid reaction represented by a pH of from 3.0 to 3.5. If the size is coagulated by an alum solution of this acidity, the colloidal and physical properties of the precipitate are injured. After the stream of size is mixed with the stream of pulp, the pH is between 6 and 8 and the pH of the pulp in the machine chest into which the uncoagulated size is discharged is between 4.0 and 5.4. In a mixture of size and pulp having a pH 10 of 6, the size does not coagulate for a long time. 15 In a mixture of size and pulp having a pH of 8 there is still free alkali, but this alkali is not absorbed by the fiber, within the time limits of contact allowed by this process.

In my process, therefore, the alum is added 20 to the pulp mixture in the machine chest in just sufficient quantity to maintain the acidity of the pulp at a pH of over 4 and preferably less than 5.4. The use of these limits contributes definitely to the efficiency of this process. As the 25 stream of stock mixed with the uncoagulated size is discharged into the machine chest, the size is very quickly and completely coagulated for the process is similar to adding a stream of size into an alum solution, where the reaction is many 30 times faster than adding a stream of alum to a size solution. This is probably the explanation why so much less alum is required when using this process.

The reason that this process is operative in 35 spite of the rapid coagulation of the size is the fact that the size is already mixed with the pulp fibers before coagulation, and the pH of the coagulating alum has been raised and the alum made more basic. Although the rate of reaction 40 between the size and alum is faster than can be successfully obtained in a beating engine, nevertheless the reactions are all uniform and under control, because the acidity of the pulp in the machine chest is uniform and under control. 45

The prior treatment of the fibers to remove all alkalinity that may be present is a step that assures the uniformity of the reaction which would not be possible if the pulp varied from an acid to an alkaline condition and it is a factor 50 in obtaining the lower alum consumption required by this process. It is evident that the chemical reaction, contemplated by this process, can not be obtained in a beater unless the beater is being fed with pulp continuously, which is seldom the case. It is also evident that this reaction can not be obtained by throwing alum and size alternately and in batches into a chest containing paper stock. The chemical reaction 55 in this process is also different from that which would be obtained by mixing together simultaneously a stream of pulp fibers, a stream of size solution, and a stream of alum solution. 60

Any kind of sizing solution may be used with 65 this process, and it is especially valuable when a size is being used that has a considerable amount of free alkali, as such a size is often very troublesome when used in beater sizing. If an ordinary size emulsion is mixed with neutral pulp, the pH of the mixture will be about 9. This 70 mixture will soon produce an alkaline fiber difficult to size, and such a size should not be mixed with the pulp more than a few seconds before it is coagulated. This is impossible to accomplish in a beater. When alum is added to such a mix- 75

ture of alkaline size and pulp in a beater, the rate of reaction is slow, requiring a large excess of alum to be used to complete the reaction and to acidify the pulp amounting generally to from 5 2% to 4% of alum by weight of the fiber.

By my process, bond and writing papers and many others can be sized with not over 1% of alum by weight of the fiber. And I also find that my process requires from one-half to one-third 10 the amount of alum generally required by present methods in beater sizing to produce the same results.

Although I have described a process where the coagulation of the size takes place in the machine chest, which is the method most suited to ordinary mill conditions, it would be possible to carry out this process by using other mixing 15 means. The size may be mixed with the pulp within the Jordan, if used, or in a small mixing device or both. The alum may be mixed with the pulp in any mixing device replacing the machine chest or a stream of alum may be added to a stream of size and pulp, provided the pH 20 of the alum solution is over 4.2 or if a very quick mixing action immediately follows. The rate of mixing of the alum solution must be proportioned to the rate of reaction between the size and alum. The rate of reaction increases as the pH is lowered. The rate of reaction is also slower as the 25 concentrations are decreased. As the pulp is transferred from the beater chest to the machine chest, there is practically no dilution of the stock, but the stock pumped from the machine chest is discharged either onto the paper 30 machine screens or into sand traps on its way to the screens, and as soon as it is discharged, it is diluted with a large amount of water being returned from the paper machine. The stock is diluted from about 3% consistency to about 40 one-half per cent consistency. The chemical reaction that takes place at one-half per cent is not completed within the time that it takes for the pulp to pass through the screens and onto the machines, and if it is attempted to coagulate 45 the size in this dilute condition, a large amount of froth is produced.

I am therefore, limiting my process to the coagulating of the size before the pulp is diluted for screening, if the ordinary paper making 50 equipment is used. My process would operate successfully, however, if a special tank were installed into which the diluted stock were discharged either before or after screening and into which the stream of alum could be poured, and 55 when the size could be coagulated and the reaction completed before the diluted pulp was pumped to the paper machine. In the case just cited, the tank above described would be a machine chest.

60 There is another modification of this process that is also important, namely, in pumping the pulp stock from the machine chest to the headbox of the paper machine, there is generally an overflow of this undiluted pulp constantly being 65 returned to the machine chest. Now, if the alum solution added for the coagulation of the size is combined with this stream of stock returning to the chest and it meets in the chest, the stream of pulp coming from the beater chest 70 containing the size, there is no chance for variations in the chemical reaction. The alum is diluted with pulp where the chemical reaction is already complete and just sufficient alum is used to maintain the pH of the solution desired 75 for proper coagulation which is generally about

4.6 although it will operate within the limits given in this specification.

I claim:

1. A method of sizing paper which comprises mixing a stream of size with a stream of non-alkaline pulp fibers; and before the fibers can absorb the alkali from the size, discharging the mixture into a chest containing pulp, precipitated size, and alum, while additional alum is continuously added to said chest. 10

2. A method of sizing paper which comprises mixing a stream of size with a stream of slightly acidified pulp fibers; and before the size is coagulated, discharging the mixture into a chest containing pulp, precipitated size and alum while 15 additional alum is continuously added to said chest.

3. A method of sizing paper which comprises mixing a stream of size with a stream of slightly acidified pulp fibers; and before the size is coagulated, discharging the mixture into a chest containing pulp, precipitated size and alum while 20 additional alum is continuously added to said chest to maintain the pH in said tank at some point between 4 and 5.2. 25

4. A step in a method of sizing paper which comprises adding a stream of paper pulp containing a mixture of slightly acidified pulp fibers and an alkaline size solution, to a chest containing acidified fiber, precipitated size and an 30 alum solution while additional alum is continuously added to said chest.

5. A method of sizing paper which includes the steps of discharging continuously a fresh mixture 35 of a weakly alkaline size and a non-alkaline pulp, into a mixing chest containing pulp fibers that are already acidified by the continuous addition of alum to a pH of between 4 and 5.2.

6. A method of sizing paper which includes the continuous addition to a chest of a mixture 40 of a non-alkaline pulp and a weak alkaline size and the continuous addition of an alum solution to the chest in sufficient quantity to coagulate the size within the chest.

7. A method of sizing paper when using pulp 45 fibers that have been prepared by an alkaline process, which comprises the steps of treating the fibers with a sufficient amount of papermakers' alum to remove the internal alkali from the fibers, then continuously adding a stream of sizing material to a stream of the pulp and before the fibers can absorb the alkali from the size, the size is coagulated by the continuous addition of a stream of alum. 50

8. A method of sizing paper pulp which includes the continuous mixing of a sizing solution with paper making fibers that have been previously slightly acidified by treatment with a fresh alum solution and immediately coagulating the size by the continuous addition of alum. 55

9. A step in the method of sizing paper pulp which comprises mixing sizing solution with a stream of pulp fibers, discharging the mixture into a mixing vat and coagulating the size in the vat by the constant addition of a stream of alum which maintains the pH in the vat at between 4 and 5.2. 60

10. A step in the method of sizing paper pulp which comprises mixing an aqueous stream of pulp fibers containing uncoagulated size with a stream of pulp fibers containing coagulated size, and alum and which is maintained at a pH of from 4 to 5.2 by the continuous addition of alum. 70